

Jan. 16, 1934.

M. M. AUSTIN

1,943,853

BIPLATE METAL

Filed Oct. 31, 1930



Inventor  
Miner M. Austin  
By Williams, Bradbury  
McCaleb & Hinke, Atty's.

## UNITED STATES PATENT OFFICE

1,943,853

## BIPLATE METAL

Miner M. Austin, Waukegan, Ill., assignor to  
 Fansteel Products Company, Inc., North  
 Chicago, Ill., a corporation of New York

Application October 31, 1930. Serial No. 492,498

4 Claims. (Cl. 29—181)

This invention relates in general to bi-plate metal, and while it pertains to bi-plate metal or roll plate such as is used in the manufacture of jewelry, the invention has more particular reference to a rare metal such as tantalum coated on an alloy of copper and a method of producing such a bi-plate metal.

While a bi-plate metal comprising a rare metal such as tantalum or columbium and a base metal 10 is desirable for use in the manufacture of rare metal articles, it is not practical to sweat or to electroplate a tantalum or columbium plate to a base metal plate in the manner now common in the case of gold and silver rolled plate, for the 15 reason, among others, that the ordinary soldering, brazing, and welding compounds and base metals will not "wet" the rare metal. Such a product of tantalum or columbium effects a saving in the quantity of rare metal required to form 20 the article, and therefore, effects a saving in the cost of the article.

The present invention contemplates dipping clean tantalum into a molten copper alloy of aluminum, nickel, or any other metal having a 25 solvent action on the tantalum. The dipping forms an adherent film or slab of the alloy on the surface of the tantalum, the film or slab protecting the tantalum surface, preventing gas absorption by the tantalum and oxidation thereof when 30 heated in air, and providing a base for the attachment of additional metal by soldering or brazing in a known manner. The copper alloys mentioned above are here preferred because of their 35 mechanical strength and resistance to corrosion.

When the film or slab has been formed on the tantalum, it is possible to proceed as in the preparation of rolled plate; that is, to attach a thick metal backing to the film or slab by means of 40 hard solder. This backing may then be annealed in air to aid in the rolling process, the film on the opposite surface of the tantalum protecting the tantalum as above described.

An important object of the invention is therefore to provide a metal plate, sheet, tube, or wire 45 of ordinary metals with an integral plate of a rare metal such as tantalum and columbium without the use of soldering compositions.

Another important object of the invention is to unite a rare metal with an ordinary metal to 50 provide a perfect joint and to eliminate bubbles or flaws in the joint thus provided, whereby to obtain perfect adhesion between the rare metal and the ordinary metal.

A further object of the invention is to provide a 55 novel means for treating rare metal plates such as

tantalum and columbium at high temperatures without the necessity of providing a vacuum or inert atmosphere.

Another object of the present invention is to provide useful and novel articles of manufacture 60 having the conductivity, strength and physical properties of copper alloy with a non-corrosive plate which has the physical, electrical and chemical characteristics of rare metals such as tantalum and columbium. 65

Still another object of this invention is the provision of a relatively inexpensive alloy and a substantially integral rare metal plate formed thereon for the manufacture of rare metal articles, whereby to effect a saving in the cost of such 70 articles.

Other objects will be apparent as the detailed description of the invention proceeds.

The accompanying drawing shows a preferred embodiment of the invention and similar parts 75 are referred to by like reference characters throughout the several views.

Fig. 1 is a horizontal section through the electric furnace and molten alloy crucible.

Fig. 2 is a perspective view of the tantalum 80 coated with an alloy film.

Fig. 3 is a horizontal section through the graphite mold in which the molten alloy is being poured.

Fig. 4 is a perspective of the strip comprising a tantalum plate having an alloy film on one side 85 and an alloy base on the other.

Fig. 5 is a diagrammatic representation of the rolling process.

Fig. 6 is a diagrammatic representation of acid 90 treating tank; and

Fig. 7 is an embodiment in which a tantalum plated wire is formed by my improved process.

Briefly the invention contemplates dipping a strip of pure tantalum metal into a super-heated bath of aluminum copper or nickel copper alloy 95 or into such bath having a layer of fused potassium tantalum fluoride covering the alloy. This coated strip is then put in a sand or graphite mold and a quantity of the alloy is poured on one side so that the strip is formed having a film of the 100 alloy on one side of the tantalum and a very thick base on the other side of the tantalum. This strip may be rolled into very thin sheets, and the adherence between the tantalum and the alloy is substantially perfect, due probably to the fact that the aluminum or the nickel in the respective alloys exerts a powerful solvent action on the tantalum.

For accomplishing the foregoing objects, a 110 graphite crucible 10 is placed in an electric fur-

nace 11, as shown in Fig. 1. This furnace may be briefly characterized as an alundum cylinder 12 having an alundum base 13 around which is wound a molybdenum coil 14, the terminals of which are connected by conductors 15 and 16 to a source of supply. Magnesia or other refractory insulating material 18 insulates the heated elements above described from the supporting frame or container 19. No novelty is claimed in the furnace per se and it will not therefore be described in detail.

The graphite crucible is nearly filled with an alloy 20 preferably of copper and nickel or copper and aluminum. The nickel content of the first alloy is preferably about 5 to 70 percent, and the aluminum in the second is from 2 to 10 percent, it being understood, however, that other percentages may be used without departing from the spirit or scope of the invention. While copper alloys are described, it will be understood that the invention contemplates the use of iron, gold, lead, platinum, aluminum, tin, and other metals. The coating or backing alloy may be characterized in general as a base metal having the desired physical and chemical properties alloyed with a solvent metal which will give perfect adhesion with tantalum.

When the alloy 20 is molten and has become slightly superheated, the temperature naturally varying with the alloy used, a strip 21 of tantalum is dipped into this molten mass to form a film on the tantalum. The strip is allowed to remain for about 15 seconds, after which it is removed from the molten alloy. This dipping forms an extremely adherent film of the alloy over the entire surface of the tantalum. The strip of tantalum coated with the alloy film is illustrated diagrammatically in Fig. 2.

A tantalum oxide film on the surface of the tantalum is sometimes responsible for the difficulties encountered in joining tantalum to a base metal. Where desired, therefore, this invention contemplates covering the molten alloy 20 with a layer of a solvent for the oxides of tantalum. A double salt of fused potassium tantalum fluoride has been found to dissolve the tantalum oxides which may have formed on the tantalum and may be used to cover the molten alloy so that the tantalum is immersed first in the upper layer of fluoride and then in the alloy therebeneath.

This strip is placed in a sand or graphite mold 22 and a relatively large amount of the alloy is poured on the strip in the mold by a crucible or ladle 23 or the coated tantalum is fixed to a thick metal backing by means of silver solder. The film 20A on the bottom of the plate remains unchanged, the film 20B on the top of the plate fuses with the added alloy 20C and becomes an integral part of this base metal. The strip of tantalum plate secured to the copper alloy base in this manner is diagrammatically illustrated in Fig. 4.

This strip may be rolled to any desired thickness by conventional rollers diagrammatically illustrated at 24 in Fig. 5. While the malleability, hardness, toughness, etc. of the tantalum differs from those qualities of the base metal, the ad-

hesion between these two metals is so great that the tantalum is reduced in thickness in the rolling process almost in proportion to the base metal. A bi-plate metal formed as described above, by continued rolling produces plates in which the tantalum is of almost microscopic thickness, and there will be no rupture between the tantalum and the base metal alloy during the entire rolling process. During the process the plate or strip may be annealed by heating it in the atmosphere, the alloy film effectively insulating the tantalum from atmospheric oxygen.

The final step of my process consists in removing the film of alloy 20A from the tantalum plate after it has been rolled to the required thickness. This film is extremely thin and may be removed by dipping the tantalum in a bath of sulphuric acid 26 or any other suitable solvent contained in a tank or receptacle 27, as shown in Fig. 3, tantalum being unattacked by practically all solvents.

By dipping a rare metal into a molten bath as described above, a coating or film of pure gold has been formed on the tantalum, and copper, silver, or lead mixed with aluminum, beryllium, or a metal of the iron group, such as nickel, when treated as described form an adherent coating on tantalum. Magnesium, calcium, silicon, or other vigorous reducing agents may be substituted for beryllium or aluminum.

Other metals and alloys suitable for coating rare metals are gold, cobalt and iron, cobalt and copper, and lead and aluminum. Instead of making flat plates of base metal alloy plated with tantalum, the molten alloy may be poured in a tantalum cylinder which has been dipped to form an alloy film as above described. This cylinder may then be swaged and drawn into a wire which will be in effect a base metal alloy core 28 surrounded by a tantalum plate 29, as shown in Fig. 7.

While a preferred embodiment of the invention has been described, it will be understood that the invention is not limited to the details set forth except as defined by the appended claims.

I claim:

1. A bi-plate metal comprising a tantalum plate, a copper alloy film thereon having from 5 to 70% nickel, and a base metal adhering to said film.

2. A bi-plate metal comprising tantalum, a copper alloy film adhering thereto and containing from 2 to 10% aluminum and a base metal adhering to said film.

3. A bi-plate article of manufacture comprising a tantalum plate, an alloy film of copper and a metal of the iron group adhering to said plate, and a base metal adhering to said film on said tantalum plate.

4. A bi-metal article of manufacture comprising a tantalum plate, a base metal film autogenously attached thereto and protecting said plate against the deleterious influences of the atmosphere, and a base metal plate autogenously attached to said film.

MINER M. AUSTIN.